

## UNITED STATES PATENT OFFICE

2,641,577

LITHIUM-CALCIUM LUBRICATING GREASE  
COMPOSITION

Rosemary O'Halloran, Roselle Park, N. J., assignor to Standard Oil Development Company, a corporation of Delaware

No Drawing. Application June 22, 1951,  
Serial No. 233,099

6 Claims. (Cl. 252—40)

1

This invention relates to lubricating compositions and more particularly to a lubricating composition containing lithium and calcium salts of a high molecular weight fatty acid.

Briefly stated, this invention comprises a superior high temperature, shear stable, moisture resistant lubricating composition made by thickening a lubricating oil to a grease consistency with a mixture of the lithium and calcium soaps of high molecular weight fatty acids in which the ratio of the lithium soap to the calcium or strontium soap is within a desired range to be given in more detail hereinafter.

The use of lithium soaps in grease making is known in the art and patents covering lithium soap grease are numerous. Lithium greases are of value for their combination of water resistance and high dropping point but are sensitive to manufacturing variables and have relatively poor shear stability. It is also known that calcium soap greases are very desirable for certain purposes, chief among which are for moisture proof lubrication, but have very poor temperature resistance.

Although lithium soap greases and calcium soap greases are well known in the art, there is very little known of a grease containing in combination a lithium soap and a calcium or strontium soap, so far as applicant is aware, and nothing at all of a grease containing a combination of the lithium soap and calcium or strontium soap of a high molecular weight fatty acid in which the ratio of lithium soap to calcium or strontium soap is within applicants desired range.

Morway in U. S. Patent 2,355,009 discloses the use of a combination of the lithium and barium soaps of fatty acids to prepare a grease composition.

Fraser, in U. S. Patent 2,397,956, teaches the manufacture of a grease using a lithium soap of 12-hydroxy stearic acid, or hydrogenated castor oil and discloses that the calcium soap of a higher fatty acid may be combined therewith, preferably as a preformed calcium grease. This combination, however, is directed toward a specific grease composition, one made with a major proportion of the lithium soap of hydrogenated castor oil. The instant application differs in other major respects as will become evident as the description proceeds.

Woods et al., in U. S. Patent 2,470,965, also teaches the manufacture of a grease composition which contains lithium soap and soluble calcium soap. Specifically, Woods et al. show the inclusion of a minor percentage of calcium naphthenate as an "anti-bleeding" agent, that

is, a substance incorporated into a grease to prevent oil separation during rapid cooling.

In a pending application, Serial No. 100,969 filed June 23, 1949, now Patent No. 2,583,435, there is disclosed a grease combining a lithium salt and a calcium soap. In this disclosure, the lithium salt is obtained by reacting lithium hydroxide monohydrate with a low molecular weight unsaturated acid.

10 The present invention comprises a grease composition combining a lithium soap and a calcium or strontium soap of a high molecular weight fatty acid. When a mixture of the lithium and calcium soaps is used, the mol ratios of the lithium soap to the calcium soap may vary between about 2:1 to 8:1, the preferred ratio being within the range of 3 mols of the lithium soap to 1 mol of the calcium soap to 6 mols of the lithium soap to 1 mol of the calcium soap.

15 20 When the amount of the lithium soap is increased beyond the 8:1 mol ratio the advantages obtained by the incorporation of the calcium soap decrease markedly, and when the amount of the calcium soap is increased above the 3:1 mol ratio, manufacturing difficulties are encountered, greater amounts of the calcium soap failing to give a grease structure that is stable.

25 30 The grease composition of this invention is an excellent all purpose lubricant, being moisture resistant and very stable to shear breakdown, having a high dropping point. The grease has a very smooth texture and a corresponding excellent appearance. It has several outstanding advantages over other greases of similar composition among which may be listed the following:

(1) Increased shear stability of major consideration in all purpose lubricants.

(2) Manufacture of the grease composition at lower temperatures. The grease of this invention may be manufactured at temperatures as low as 320° F. Other lithium based greases must be made at temperatures as high, in some instances, as 430° F.

(3) Less sensitivity to manufacturing variables. 45 For example, the greases of this invention made from oils having a high viscosity index may be cooled in thick layers or "cakes" whereas lithium based greases must be "pan cooled" or cooled in thin layers. This advantage is obvious.

(4) A decreased amount of aeration upon being subjected to mixing or shear stresses. This is of particular importance when used in high speed bearing surfaces since the incorporation of air into a lubricant under those conditions 50 decreases the lubricating potential.

(5) An increased resistance to the solvent ac-

2

tion of hydrocarbons. This permits the use of the grease of this invention as a lubricant for surfaces exposed to action of hydrocarbon solvents with improved performance.

Although the greases of this invention may be made from any of the usual natural or synthetic grease-forming fats or fatty acids such as oleic acid, stearic acid, resin acids, beef fat, tallow or the saturated or unsaturated glycerides of various fatty acids, Fischer-Tropsch residues, or mixtures of the above, the preferred embodiment contemplates the use of high molecular weight fatty acids and particularly the high molecular weight substantially saturated acids such as the hydrogenated fish oil acids.

The lubricating oils into which the soaps are incorporated according to this invention may be any of the numerous types of lubricating oils, whether natural or synthetic and may have viscosities of from 60 to 4000 Saybolt seconds at 100° F. Preferably, however, the greases of this invention are made using as a base oil a naturally occurring mineral oil distillate.

Any of the conventional methods of manufacture such as cooking in a fire heated kettle followed by drawing into thin pans or deep cakes for cooling, or, due to the lower maximum temperature required to form the greases of this invention, they may be manufactured in the conventional steam heated kettles at a maximum of 325° F. in some cases, followed by cooling with stirring while running cold water through the kettle jacket.

The concept of this invention may be more clearly explained by reference to the following examples, which, it is understood, are to be taken as illustrative only.

#### EXAMPLE 1

The following formulation was used in the preparation of a series of greases according to the instant invention.

15.00% of hydrogenated fish oil acids having a saponification value of from 195 to 215 was used with .06 mol equivalents of base consisting of a mixture of lithium and calcium hydroxides, the percentages of the base being adjusted to give the desired molar ratio of lithium soap to calcium soap. The balance of the formulation consisted of the desired base oil and included 0.50% of an oxidation inhibitor such as phenyl-alpha naphthylamine.

The procedure used for the manufacture of the grease compositions was as follows:

The fatty acid and one-fifth of the mineral oil were charged to a steam heated grease kettle and heated to 150° F. The calcium hydroxide in the form of a water slurry was added and the mass cooked for five minutes. After the cooking a boiling water solution of the lithium hydroxide was added and the mixed soap mass dehydrated for one-half hour at 200 to 230° F. The mass was then raised to a temperature of about 300° F., during which the remainder of the oil charge was added in small amount. The temperature was again raised until the product was completely fluid. At this point, the oxidation inhibitor was added. (At this point, also, other materials such as "defoamers" can be added.) The product was then poured into cooling equipment and allowed to cool to room temperature.

Various inspection tests were performed on the grease compositions manufactured according to the formulation and procedure described above. For examination of their structure stability and

shear resistance the greases were subjected to the worker test. The ASTM dropping points were also taken. These tests were conducted according to standard procedures, and the results are shown in Table I below:

Table I  
INSPECTION TESTS ON LITHIUM-CALCIUM GREASES

| Mol Ratio | Dropping Point (° F.) | Cooling Method | Worker Tests, Using Fine Hole Plate, Penetration (mm./10) |                      |
|-----------|-----------------------|----------------|-----------------------------------------------------------|----------------------|
|           |                       |                | After 1,000 Strokes                                       | After 60,000 Strokes |
| 15        |                       |                |                                                           |                      |
| 18:1      | 371                   | Thin Layer     | 261                                                       | 337                  |
|           |                       | Cake           | 319                                                       | (not run)            |
| 8:1       | 359                   | Thin Layer     | 276                                                       | 346                  |
|           |                       | Cake           | 335                                                       | (not run)            |
| 6:1       | 368                   | Thin Layer     | 308                                                       | 341                  |
|           |                       | Cake           | 312                                                       | 343                  |
| 4:1       | 330                   | Thin Layer     | 288                                                       | 326                  |
|           |                       | Cake           | 286                                                       | 333                  |
| 3:1       | 346                   | Thin Layer     | 305                                                       | 347                  |
|           |                       | Cake           | 319                                                       | 364                  |
| 2:1       | 297                   | Thin Layer     | 317                                                       | (not run)            |
|           |                       | Cake           | 335                                                       | Do.                  |

An examination of the above table will serve to illustrate the outstanding characteristics of the greases of this invention particularly with regard to shear stability and lack of sensitivity to cooling methods in case of the grease representing the optimum ratio.

#### EXAMPLE 2

A specific example of a grease composition made in accordance with the procedure outlined in Example 1 above and containing the optimum ratio of soaps had the following percentage composition, all percentages being by weight based on the total composition.

| Per cent                                                                           |
|------------------------------------------------------------------------------------|
| Hydrogenated fish oil acids having a saponification value of 212                   |
| 15.00                                                                              |
| Lithium hydroxide monohydrate                                                      |
| 1.73                                                                               |
| Calcium hydroxide (68.0% CaO)                                                      |
| 0.82                                                                               |
| Phenol extracted coastal distillate having a viscosity at 210° F. of 37 S. U. S.   |
| 12.40                                                                              |
| Phenol extracted Panhandle Distillate having a viscosity at 210° F. of 44 S. U. S. |
| 69.21                                                                              |
| Phenyl-alpha naphthylamine                                                         |
| 0.50                                                                               |
| Free acidity calculated as oleic acid (ASTM—D128-47 method)                        |
| 0.34                                                                               |

#### EXAMPLE 3

A grease directly suitable for multi-purpose industrial service, especially where satisfactory lubrication of both automotive and other industrial equipment is required from a single lubricant, may be prepared by applying the concept of this invention to a lithium-calcium grease dispersed in a coastal distillate of relatively high viscosity, i. e., of approximately 500 S. U. S. at 100° F.

An example of such grease was prepared according to the following formula using the procedure outlined in Example 1 above:

| Per cent                                                                      |
|-------------------------------------------------------------------------------|
| Hydrogenated fish oil acids                                                   |
| 12.50                                                                         |
| Lithium hydroxide monohydrate                                                 |
| 1.42                                                                          |
| Calcium hydroxide                                                             |
| 0.67                                                                          |
| Acid treated coastal distillate having a viscosity at 100° F. of 500 S. U. S. |
| 85.41                                                                         |

In laboratory tests considered significant in the evaluation of industrial and automotive greases, a grease of the above composition shows superior performance in several respects to that

of a lithium stearate based grease prepared in the same mineral oil. The lithium stearate grease required a manufacturing temperature 75° F. higher than the grease of this invention, a consideration of major economic and safety concern.

Table II  
MULTI PURPOSE LITHIUM-CALCIUM GREASE

| Shear Stability Properties                               | Lithium-Calcium Grease (Ex. 3) | Lithium Grease |
|----------------------------------------------------------|--------------------------------|----------------|
| Penetration, mm./10:                                     |                                |                |
| Unworked.....                                            | 296.....                       | 290.....       |
| 60 strokes.....                                          | 294.....                       | 295.....       |
| 60,000 strokes (Fine Hole).....                          | 325.....                       | 335.....       |
| Balcrank Dispensing Rate, g./min. at 77° F. <sup>1</sup> |                                |                |
| Micropenetration, mm./10, Before.....                    | 51.....                        | 53.....        |
| Micropenetration, mm./10, After.....                     | 107.....                       | 121.....       |
| High Temperature Properties:                             |                                |                |
| Dropping Point, ° F.....                                 | 345.....                       | 390.....       |
| Oil Separation, Percent Loss, 50 Hrs./210° F.....        | 1.4.....                       | 2.1.....       |
| Wheel Bearing Test (AXS-1574) at 220° F.....             | Pass.....                      | Pass.....      |
| Oil Leakage, grams.....                                  | None.....                      | Trace.....     |
| Water Resistance:                                        |                                |                |
| Water Wash, Percent Loss at 77° F.....                   | 7.5.....                       | 5.0.....       |
| Emulsion in Water at 212° F. (Army 2-134).....           | None.....                      | None.....      |

<sup>1</sup> Grease dispensed through a shackle having a .0003 inch clearance at 100 p. s. i. g. pressure and at a flow rate of 50 gms./min. resulting in a shear rate of approx. 20,000 sec.<sup>-1</sup>.

An examination of the data in Table II above shows the superiority of the grease of this invention to the straight lithium base grease in regard to shear stability (325 vs. 335 after 60,000 strokes) and shows less breakdown on dispensing through the Balcrank grease gun under high rates of shear. Somewhat superior resistance to oil separation at elevated temperatures is shown for the lithium-calcium grease (1.4% vs. 2.1% at 210° F.). Oil separation after the Ford wheel bearing test was also observed in the lithium base grease but none in the lithium-calcium grease.

#### EXAMPLE IV

As an illustration of a grease made from a synthetic oil base, a grease having the following composition was prepared:

|                                  | Per cent |
|----------------------------------|----------|
| Calcium stearate .....           | 5.00     |
| Lithium stearate .....           | 10.00    |
| Phenyl alpha naphthylamine ..... | 0.50     |
| Di-2-ethylhexyl sebacate.....    | 84.50    |

The dry preformed soaps were admixed with the synthetic ester base and heated to 350° F., drawn into pans for cooling and then homogenized. The product was smooth in appearance and equivalent in shear stability to a conventional grease prepared from straight lithium stearate.

It is to be understood, of course, that various additives known to the art such as extreme pressure additives, anti-corrosion agents, viscosity in-

dex improvers, and the like, may be incorporated into these grease compositions to increase their desirable characteristics.

In summation, this invention comprises a new and superior grease composition having properties that make it outstanding for a general, all purpose lubricant which consists essentially of a lubricating oil that is thickened to a grease consistency with the lithium soap and the calcium or strontium soap of a high molecular weight fatty acid in which the molar ratio of the lithium soap to the calcium or strontium soap varies within the range of from 2:1 to 8:1, preferably 3:1 to 6:1.

What is claimed is:

1. A lubricating composition which comprises a lubricating oil thickened to a grease consistency with a mixture of the lithium and calcium soaps of an unsubstituted substantially saturated high molecular weight saponifiable material wherein the molar ratio of the lithium soap to the calcium soap is within a range of from 6:1 to 3:1.

2. A lubricating composition which comprises a lubricating oil thickened to a grease consistency with a mixture of the lithium and calcium soaps of an unsubstituted substantially saturated high molecular weight saponifiable material wherein the molar ratio of the lithium soap to the calcium soap is 4:1.

3. A lubricating composition according to claim 1 in which the high molecular weight saponifiable material is a hydrogenated fish oil acid.

4. A lubricating composition according to claim 2 in which the fatty acid is a hydrogenated fish oil acid.

5. A lubricating composition having the following formulation in which the percentages are by weight based on the total compositions:

|                                                                                    | Per cent |
|------------------------------------------------------------------------------------|----------|
| Hydrogenated fish oil acids .....                                                  | 12.50    |
| Lithium hydroxide monohydrate .....                                                | 1.42     |
| Calcium hydroxide .....                                                            | 0.67     |
| Acid treated coastal distillate having a viscosity at 100° F. of 500 S. U. S ..... | 85.41    |

6. A composition according to claim 1 in which the lubricating base is di-2-ethylhexyl sebacate.

ROSEMARY O'HALLORAN.

#### References Cited in the file of this patent

#### UNITED STATES PATENTS

| Number    | Name               | Date           |
|-----------|--------------------|----------------|
| 2,293,052 | Earle .....        | Aug. 18, 1942  |
| 2,318,847 | Flint .....        | May 11, 1943   |
| 2,355,009 | Morway .....       | Aug. 1, 1944   |
| 2,403,104 | Lien .....         | July 2, 1946   |
| 2,450,221 | Ashburn .....      | Sept. 28, 1948 |
| 2,497,133 | Morway .....       | Feb. 14, 1950  |
| 2,583,435 | Morway .....       | Jan. 22, 1952  |
| 2,588,556 | Moore et al. ..... | Mar. 11, 1952  |